

# UNITED STATES PATENT OFFICE.

WILLIAM H. ALLEN, OF DETROIT, MICHIGAN, ASSIGNOR TO PARKER RUST-PROOF COMPANY OF AMERICA, OF DETROIT, MICHIGAN, A CORPORATION OF MICHIGAN.

## PROCESS FOR RUST-PROOFING METAL.

1,215,463.

Specification of Letters Patent. Patented Feb. 13, 1917.

No Drawing.

Application filed November 6, 1915. Serial No. 60,072.

To all whom it may concern:

Be it known that I, WILLIAM H. ALLEN, a citizen of the United States, residing at Detroit, in the county of Wayne and State 5 of Michigan, have invented a new and useful Process for Rust-Proofing Metal, of which the following is a specification.

This invention relates to the process of so acting upon the surfaces of articles of iron 10 and steel as to render them rust-proof, that is, to so change the character of such surfaces that they will be substantially unaffected upon exposure to moist air. This invention is carried out by changing such surfaces into insoluble basic phosphate of iron 15 by immersing the articles in a proper bath, hereinafter described, at substantially the boiling point, which surface will thereafter resist the corroding action of the atmosphere.

Ferric phosphate may be prepared in any well known manner, but I prefer to add to a solution of a soluble phosphate, such as sodium phosphate, a solution of a ferric salt, 20 such as ferric sulfate or chlorid, which causes a precipitation of ferric phosphate. The reaction may be written



30 This precipitate is then washed to remove the soluble sodium salt. The ferric phosphate is then dissolved in phosphoric acid which results in the formation of ferric acid 35 phosphate.



A substantially eight-tenths per cent. solution of this ferric acid phosphate in water 40 is brought to about the boiling point and the articles of iron and steel to be treated are then placed therein, whereupon probably the following reaction occurs.



The surfaces of the iron and steel become black as the basic phosphates of iron are

formed, the action of the bath being continued until hydrogen ceases to escape, after 50 which the articles are removed from the bath and are then dried and oiled.

It will be noticed that no free phosphoric acid is introduced in the bath, which is a solution of a phosphate or salt. The affected 55 surfaces of the iron or steel are integral with the body of the article and after the treatment is completed there is no tendency of the surfaces to separate from the main body of the article. The bath may be continued in use until it is exhausted or be kept up to standard strength through the addition of fresh ferric acid phosphate.

One of the prime advantages of this invention lies in the fact that the ferric acid 65 phosphate can be shipped to the factories where rust-proofing is to be carried out, where it can be added to the bath as required, thus avoiding the mistakes that are liable to occur where unskilled labor is employed to mix the ingredients of previous 70 rust-proofing baths.

The exact composition of the ferric acid phosphates is uncertain, as these compounds vary greatly from



I therefore do not wish to be understood as 80 vouching for the accuracies of the reactions given above.

I claim:

1. The process of rendering articles of iron and steel rust-proof which consists in immersing the same in a solution of ferric acid 85 phosphate.

2. The process of rendering articles of iron and steel rust-proof which consists in immersing the same in a substantially boiling 90 bath of water containing about eight-tenths per cent. of ferric acid phosphate.

In testimony whereof I sign this specification.

WILLIAM H. ALLEN.